

## UNITED STATES PATENT OFFICE

2,611,689

## ARTICLE FOR POLISHING

Philip W. Porter, Higganum, Conn., assignor to  
 D. & H. Scovil, Inc., Higganum, Conn., a corpora-  
 tion of Connecticut

No Drawing. Application September 6, 1949,  
 Serial No. 114,275

9 Claims. (Cl. 51—298)

1

This invention relates to a polishing layer and to a method for preparing the layer. More particularly, the invention relates to a polishing layer which comprises finely divided abrasive particles imbedded in an adhesive matrix which exhibits characteristics of fluidity, resilience and lubricity which make the composition uniquely suitable for use in the manufacture of polishing implements such as polishing wheels and polishing belts which are normally operated at high speed in frictional engagement with surfaces which it is desired to polish.

As it is well understood, commercial finishing of articles of manufacture, both ferrous and non-ferrous, is ordinarily accomplished by maintaining the surface of the article in frictional engagement with an endless surface, such as that provided by a wheel or an endless belt, which is coated with an abrasive layer which acts to reduce the irregularities on the surface of the article. The surface of the article is acted on successively by abrasive particles of increased fineness and the final, or polishing operation, is accomplished with an extremely fine abrasive material such as rouge.

It has been observed frequently that an adhesive matrix, the adhesive composition in which the abrasive particles are imbedded and which adheres to the endless surface provided by a belt or wheel, which is entirely suitable for retaining larger abrasive particles in polishing position on the surface of the belt or wheel is not satisfactory for polishing purposes as differentiated from cutting or surface removal purposes. Most heavy surface removal is accomplished with grains larger than 100 mesh, and polishing is accomplished with grains smaller than 100 mesh. Silicate base binding cements are generally limited to use with 100 mesh grains and larger, as it is recognized that such silicate base cements are not sufficiently resilient to permit the abrasive particles to retreat into the film and permit polishing action, which is accomplished partially by a plastic flow of the metal induced by the polishing action of the abrasive layer. Animal glues, on the other hand, make a satisfactory matrix for fine abrasive particles, but the use of animal glues in the manufacture of a polishing device entails several practical difficulties. For example, animal glue employed as an abrasive particle matrix must be cured within a certain range of temperature and humidity conditions, and it will decay if it is exposed to the atmosphere for any considerable period of time.

The object of this invention is to provide a

2

polishing layer comprising finely divided abrasive particles and an adhesive matrix which is characterized by a fluidity, resilience and lubricity which effectively retains the fine abrasive particles against displacement and which is chemically stable during long periods of storage or exposure to the atmosphere.

A further object of the invention is to provide an adhesive matrix for fine abrasive particles which may be worked at normal temperatures and which can be cured under normal atmospheric conditions without impairing its effectiveness.

Heretofore, with the two most common manufactured abrasive grains, silicate base cements have been used effectively only with aluminum oxide abrasive grains, and they have not proven to be satisfactory for bonding silicon carbide grains, apparently as a result of the evolution of gas occurring when the carbide grains are used with silicate base adhesives which prevents effective bonding of the carbide grains. It will be apparent, therefore, that the instant adhesive matrix which does not exhibit this reaction to silicon carbide grains will substantially increase the usefulness of carbide grains in the preparation of polishing implements for use on non-ferrous metals, and articles of small sizes, or on those having hard surfaces.

It has been found that an adhesive matrix having excellent properties with respect to retaining a finely divided abrasive material in polishing position on the endless surface of a wheel or belt which is operated at speeds which develop a high frictional heat can be formulated, by a method described more particularly hereinafter, from certain proportions of a synthetic resin and an alkali-silicate and certain diluents which act to stabilize the matrix and enhance its workability. The adhesive character of the matrix is imparted by the synthetic resin and the alkali-silicate, and the diluents which are added increase the chemical stability, prevent hardening during extended periods of storage and increase the workability. These diluents comprise a polyhydric alcohol which apparently acts to modify the adhesive constituents as well as acting as a plasticizer and smoothing agent which prevents premature hardening of the matrix. The diluents also include a kaolin type clay of extremely fine particle size, and a carboxymethylcellulose ester which is slightly alkaline in solution which prevents premature breaking of the emulsion of the synthetic resin when, as it is most convenient, the synthetic resin employed is in the form of an

oil-in-water type emulsion. Additionally, the carboxymethylcellulose ester also appears to improve the flexibility of the film deposited from a solution of the instant adhesive matrix.

Polyvinyl acetate is one of the synthetic resins which is suitable for use in practicing the instant invention. The polyvinyl acetate may be employed conveniently in emulsion form. The manner in which the emulsion is prepared appears to be immaterial. It may, for example, be prepared by first polymerizing the acetate monomer and thereafter dispersing the polymerized vinyl acetate in water, or as described in detail in U. S. Patent No. 2,401,445 to White, dated June 4, 1946, be prepared by carrying out the polymerization in a dispersion of the monomeric acetate. A commercially available emulsion of polyvinyl acetate resin having a solid content of about 56% has proved to have the optimum proportion of resinous material for the fluidity required for ease of handling. It will be understood, however, that in the following examples and in the claims the emulsions referred to may be diluted or dehydrated within a reasonable limit without departing from the scope of the invention.

The alkali silica found to be most effective in preparing the instant composition has an alkali to silica ratio of about 1 to 3. A sodium silicate of this character is an opalescent, syrupy liquid of relatively low alkalinity and has a specific gravity of about 1.4. Good results are obtained, however, with other alkali-silicates.

A suitable carboxymethylcellulose may be obtained by reacting sodium monochloroacetate with alkali cellulose and substituting approximately .75 carboxymethyl group for each anhydro glucose unit in the resulting sodium carboxymethylcellulose molecule. Commercially available grades of this ingredient produce good results.

The character of the clay which is used as a filler in the instant matrix effects importantly the character of the matrix. The essential requirement of a satisfactory clay is extremely small particle size. A kaolin type of clay having a screen residue on a 325 mesh screen of less than .2%, indicating a particle size of less than 2 microns in over 80% of the clay, has been found to be satisfactory consistently. A clay of this type is comprised principally of silica, alumina and a small amount of iron oxide.

Effectiveness as an adhesive matrix for abrasive particles of less than 100 mesh is limited to compositions which comprise only certain proportions of the named ingredients. Although the workable proportions of each ingredient is not sharply defined, the critical proportions appear to be, by weight, from about 4 to 36% of polyvinyl acetate water emulsion having a solid content of about 56%, 65 to 40% alkali-silicate, .5 to 6% sodium carboxymethylcellulose, 26 to 16% clay, and 4.5 to 2.0% polyhydric alcohol. Any marked reduction in the proportion of polyhydric alcohol, sorbitol being the most effective, will cause the adhesive composition to harden prematurely in shipping containers or upon extended exposure to the atmosphere. An increase in the amount of polyvinyl acetate resin beyond the maximum specified will not materially increase the strength of the film deposited from a solution of the adhesive composition, and due to the increased free acetic acid present in the larger amount of polyvinyl acetate emulsion an increased amount of sodium carboxymethylcellulose may be required to neutralize the composi-

tion. However, increased quantities of the sodium carboxymethylcellulose weakens the bond strength of the composition. Excesses of sorbitol beyond the proportion specified also reduce the tensil strength and render too plastic the film deposited from a solution of the adhesive composition.

Although no satisfactory explanation has been developed, the order in which the ingredients are admixed is a critical factor in obtaining a satisfactory adhesive matrix. Otherwise, there are no limiting conditions; good results are obtained by carrying out the process under normal conditions of atmospheric temperature and pressure. Illustrating the method of preparing the adhesive matrix by way of example:

#### Example 1

15 pounds of alkali-silicate (sodium silicate) was placed in a mixing container and agitated by a revolving beater running at medium speed. 6 pounds of kaolin clay was added gradually and the mixing continued until the mixture was smooth. 1 pound of sorbitol was added and the mixing continued until the sorbitol appeared to be homogeneously dispersed throughout the composition. 1½ pounds of sodium carboxymethylcellulose was added and the beating continued. Thereafter 6 pounds of polyvinyl acetate water emulsion having about a 56% solid content was added. This addition caused the composition to thicken, and the beating was continued until the composition appeared to have a uniform density. Thereupon, an additional 6 pounds of acetate emulsion was added and the beating continued at medium speed for about 20 minutes. At the end of this period the composition appeared to be homogeneous and of uniform density. The composition was then drawn off into shipping containers and allowed to stand exposed to atmospheric conditions for several weeks. No hardening occurred; the composition proved to be as effective after storage as it was at the time it was freshly drawn from the mixing container.

The solution of the matrix was applied to the surface of an endless fabric belt and thereafter the belt was rolled in contact with finely divided abrasive particles of about 220 mesh. The belt was allowed to cure for 24 hours under normal atmospheric conditions. The belt was then tested for polishing qualities comparatively with belts having abrasive particles of the same size imbedded, respectively, in an animal glue matrix, an artificial resin matrix and a silicate base glue matrix. The belt treated with the composition prepared according to the foregoing example proved to be superior in maintaining the fine abrasive particles in polishing engagement with the article being finished as well as having superior flexibility which permitted a greater area of the face of the belt to be maintained in contact with the article being finished. The lubricity of the composition greatly improved the heat resistance of the belt and the belt was found to wear three to four times longer than the others tested. The quality of the polishing was improved due to the tendency of the instant composition to release the larger abrasive particles, rather than retain them as an animal glue would tend to do and cause the surface of the article being finished to be burnished. The improved resiliency of the adhesive matrix also contributed to a higher quality polishing as minute irregularities on the surface of the article being finished appeared to be peened over into adjacent

deprivities rather than torn off by the abrasive particles as would occur if the matrix in which the particles were imbedded did not yield to some extent to the irregularity on the surface of the article.

Other preparations of the composition which proved to be equally effective were made as follows:

*Example 2*

The same method of preparation was followed as outlined in the foregoing example, using by weight a total of 9 parts polyvinyl acetate water emulsion, 15 parts alkali-silicate, 6.0 parts clay, 1.0 part sodium carboxymethylcellulose and 1.0 part sorbitol.

The adhesive composition thus prepared was made up in the manner prescribed in the foregoing example. In this instance, however, silicon carbide abrasive particles of about 100 mesh were added directly to the solution and the solution thereafter applied to the endless surfaces of a belt and wheel. The quality of polishing obtained with the belt and wheel thus prepared was uniformly superior.

*Example 3*

The same procedure outlined in Example 1 was followed using 15 pounds of sodium silicate, 6 pounds of clay, 1 pound of sorbitol,  $\frac{3}{4}$  pound sodium carboxymethylcellulose, and a total of 6 pounds of polyvinyl acetate water emulsion having about 56% solid content.

The composition thus prepared was stored in shipping containers for several weeks without impairing the effectiveness of the composition.

*Example 4*

The procedure outlined in Example 1 was again followed, using 15 pounds of sodium silicate, 6 pounds of clay, 1 pound of sorbitol,  $\frac{1}{2}$  pound of sodium carboxymethylcellulose and a total of 4 pounds of polyvinyl acetate water emulsion having about 56% solid content.

The composition thus prepared was tested in the same way as that described in Example 1. The results were equally good.

*Example 5*

The procedure outlined in Example 1 was followed using 15 pounds of sodium silicate, 6 pounds of clay, 1 pound of sorbitol,  $\frac{1}{4}$  pound of sodium carboxymethylcellulose and a total of 2 pounds of polyvinyl acetate water emulsion having about 56% solid content. The composition thus described was tested in the same manner as that described in Example 1 with equally satisfactory results.

*Example 6*

The procedure outlined in Example 1 was followed using 15 pounds of sodium silicate, 6 pounds of clay, 1 pound of sorbitol,  $\frac{1}{8}$  pound of sodium carboxymethylcellulose and a total of 1 pound of polyvinyl acetate water emulsion having about 56% solid content. This composition was tested in the same manner as that described in Example 1 using abrasive particles of about 100 mesh.

It was noted that all the adhesive matrices within the prescribed limits of composition satisfactorily bond all sizes of abrasive grains, from the heaviest to the lightest. In this instance a high quality polishing was obtained with the belts treated with the described polishing layer.

As it is indicated in the foregoing examples,

the composition prepared according to the invention is water soluble which makes it safe and easy to handle and facilitates resurfacing the wheels, drums, belts or paper to which the polishing composition has been applied. It will also be apparent that the adhesive matrix may be applied to the surface first and the abrasive later dusted or rolled into the adhesive, or the adhesive matrix may be mixed with the abrasive particles, such as, for example, silicon carbide or aluminum oxide, to form a polishing layer which is thereafter applied to the surface which is to be treated. Furthermore, several layers of polishing material may be built up one upon the other so that when the uppermost layer is worn off the under layer will present a polishing surface.

It will be apparent that the character of the adhesive matrix may be modified to some extent to meet various particular requirements by the addition of various well known plasticizers and fillers which act to alter the smoothness, flexibility or toughness of the film deposited is well understood in the art.

If it is desired, for example, to produce a polishing implement which is suitable for working under water in a wet polishing process, the water resistance of the adhesive matrix may be increased by the addition of glyoxyl, cupric glychromate, sodium glychromate, chromic acetate, and, or alternately, heating the polishing layer to a temperature of about 125° centigrade for several minutes to cause a fusion of the resin.

Having thus described the invention, what is new and desired to be secured by Letters Patent is:

1. A matrix for abrasive particles comprising by weight, 4 to 36% of polyvinyl acetate water emulsion having a solid content of about 56%, 65 to 40% alkali-silicate, .5 to 6% sodium carboxymethylcellulose, 26 to 16% clay, and 4.5 to 2.0% sorbitol.
2. A matrix for abrasive particles comprising by weight 9 parts polyvinyl acetate water emulsion having about 56% solid content, 15.0 parts alkali-silicate, 6.0 parts clay, 1.0 part sodium carboxymethylcellulose and 1.0 part sorbitol.
3. A matrix for abrasive particles comprising by weight 4.0 parts polyvinyl acetate water emulsion having about 56% solid content, 15.0 parts alkali-silicate, 6.0 parts clay, .5 part sodium carboxymethylcellulose, and 1.0 part sorbitol.
4. A matrix for abrasive particles comprising by weight 1.0 part polyvinyl acetate water emulsion having about 56% solid content, 15.0 parts alkali-silicate, 6.0 parts clay, .1 part sodium carboxymethylcellulose and 1.0 part sorbitol.
5. A composition for depositing a polishing layer comprising abrasive particles dispersed in an adhesive composition comprising by weight 4 to 36% of polyvinyl acetate water emulsion having a solid content of about 56%, 65 to 40% alkali-silicate, .5 to 6% sodium carboxymethylcellulose, 26 to 16% clay, and 4.5 to 2.0% sorbitol.
6. A composition for depositing a polishing layer comprising abrasive particles dispersed in an adhesive matrix comprising by weight 12 parts polyvinyl acetate water emulsion having about 56% solid content, 15 parts alkali-silicate, 6.0 parts clay, 1.5 parts sodium carboxymethylcellulose and 1.0 part sorbitol.
7. A composition for depositing a polishing layer comprising abrasive particles dispersed in an adhesive matrix comprising by weight 6.0 parts polyvinyl acetate water emulsion having about 56% solid content, 15.0 parts alkali-silicate, 6.0

parts clay, .75 part sodium carboxymethylcellulose and 1.0 part sorbitol.

8. A composition for depositing a polishing layer comprising abrasive particles dispersed in an adhesive matrix comprising by weight 2.0 parts polyvinyl acetate water emulsion having about 56% solid content, 15.0 parts alkali-silicate, 6.0 parts clay, .25 part sodium carboxymethylcellulose, and 1.0 part sorbitol.

9. A polishing implement comprising a body having a flexible surface, a polishing layer adhering to said surface, said layer including abrasive particles dispersed in an adhesive matrix comprising by weight about 2.24 to 20% of polyvinyl acetate, 65 to 40% alkali-silicate, 5 to 6% sodium carboxymethylcellulose, 26 to 16% clay, and 4.5 to 2.0% sorbitol.

10 PHILIP W. PORTER.

#### REFERENCES CITED

The following references are of record in the file of this patent:

##### UNITED STATES PATENTS

| Number    | Name          | Date          |
|-----------|---------------|---------------|
| 2,111,272 | Paulson       | Mar. 15, 1938 |
| 2,124,055 | Courtney      | July 19, 1938 |
| 2,465,295 | Strauss       | Mar. 22, 1949 |
| 2,486,756 | Murphy et al. | Nov. 1, 1949  |

##### FOREIGN PATENTS

| Number   | Country       | Date          |
|----------|---------------|---------------|
| 1462,697 | Great Britain | Mar. 15, 1937 |